

Dec. 29, 1959

K. SCHÖLZEL

2,919,207

METHOD OF APPLYING A FERROMAGNETIC SURFACE TO A BASE  
UTILIZING IRON CARBONYL AND OXYGEN

Filed Jan. 24, 1956



INVENTOR.

KARL SCHÖLZEL

BY  
*Kenway, Jenney, Winter & Aldred*

ATTORNEYS

## 1

2,919,207

## METHOD OF APPLYING A FERROMAGNETIC SURFACE TO A BASE UTILIZING IRON CARBONYL AND OXYGEN

Karl Schörlzel, Frankfurt am Main, Germany, assignor to Max Braun, Frankfurt am Main, Germany, a partnership

Application January 24, 1956, Serial No. 561,124

## 2 Claims. (Cl. 117—106)

The present invention relates to magnetic recording materials, such as those commonly used for the recording of sound. In particular, the invention provides an improved magnetic recording material and a novel method of applying extremely thin substantially homogenous ferromagnetic coatings to an appropriate base material which will generally be a non-magnetizable tape, disk, cylinder or structure of other suitable form.

Magnetic recording materials of this type are well-known commodities and have been made in the past by one of several techniques. Most commonly a very finely divided ferromagnetic material is combined with a binder material which coats the base surface. Another technique consists in applying a thin foil of the ferromagnetic material to the base surface. Use has also been made of electrodeposition, spray coating, coating by evaporation under vacuum, and coating by cathode sputtering. The better of these processes are rather complicated and require costly apparatus and delicate controls, and those more easily carried out do not generally yield a high quality product. By the present invention, on the other hand, a ferromagnetic coating may very easily and accurately be applied to produce a uniform recording material of very high quality. In general, the process consists in depositing the ferromagnetic coating on the surface by thermally decomposing in situ the carbonyl of the desired metal.

Carbonyl compounds are known for numerous metals which are either magnetizable or useful in forming magnetizable alloys such as iron, nickel, cobalt, and molybdenum, these metals being among the most important constituents of magnetizable substances. These compounds may be converted to vapor form in which they are stable up to a temperature at which they decompose to yield the metal. The present invention takes advantage of this behavior, and is carried out by exposing the surface of the base material, at decomposition temperature, to the desired carbonyl compound in gaseous form. The carbonyl compound is thereupon decomposed at the surface of the base material to form a homogeneous coating of the magnetizable metal.

The nature of the coating can easily be controlled by varying the concentration and pressure of the vapors of carbonyl compound, and by controlling the time and temperature of exposure. Since the concentration, and pressure over the entire area subject to exposure is quite uniform, and since time and temperature conditions are readily controllable, it will be appreciated that extremely consistent and accurately controlled coatings may be formed without the aid of binder materials.

Suitable carbonyl compounds are listed in Table I, which also gives their boiling points and decomposition temperatures at atmospheric pressure. These compounds are defined herein as metallic carbonyl compounds of the Werner type, since they are formed by covalent (Werner) bonding of CO, alone or with other groups, to the metal.

2  
Table I

|    | Carbonyl compound                                             | Vapor pressure mm Hg at °C | Decomposition temp. °C |
|----|---------------------------------------------------------------|----------------------------|------------------------|
| 5  |                                                               |                            |                        |
|    | Iron pentacarbonyl, Fe(CO) <sub>5</sub>                       | 15 at 25°                  | 150                    |
|    | Nickel carbonyl, Ni(CO) <sub>4</sub>                          | 261 at 15°                 | 60                     |
|    | Cobalt nitrosyl carbonyl, Co(NO)(CO) <sub>4</sub>             | 56 at 16°                  | 100                    |
|    | Cobalt carbonyl hydride, Co(CO) <sub>4</sub> H                | Very volatile              | -33                    |
| 10 | Iron nitrosyl carbonyl, Fe(NO) <sub>2</sub> (CO) <sub>3</sub> | 4.5 at 0°                  | 50                     |
|    | Iron carbonyl hydride, Fe(CO) <sub>4</sub> H <sub>2</sub>     | 11 at -10°                 | -33                    |
|    | Molybdenum carbonyl, Mo(CO) <sub>6</sub>                      | 2.3 at 55°                 | 150                    |

From Table I it will be seen that numerous carbonyl compounds are available for use in this invention, including not only carbonyls, but also nitrosyl carbonyls and carbonyl hydrides. The carbonyls, e.g. iron pentacarbonyl, may be used alone or in admixture with other carbonyl compounds to give a ferromagnetic coating of controlled variable composition. Thus, the coating may be iron or a mixture of iron and one or more other metals, e.g. cobalt, nickel and molybdenum.

Oxide coatings may also be formed by this invention by decomposing the carbonyl, e.g. iron pentacarbonyl, on the base surface in the presence of oxygen.

15 As base materials, any non-magnetizable material which is stable at the temperatures encountered during deposition of the ferromagnetic material, and which may be formed with a smooth surface may be used. Particularly useful are paper and flexible organic plastic film-forming materials such as polyvinyl chloride, vinyl chloride-vinyl acetate copolymers, vinylidene chloride, vinylidene chloride-vinyl chloride copolymers, polyvinyl alcohol, polyethylene, polytetrafluoroethylene, polychlorotrifluoroethylene, polystyrene polyamides, rubber hydrochloride, vinyl nitrile rubber, regenerated cellulose, cellulose acetate, cellulose triacetate, cellulose acetate butyrate, cellulose nitrate, ethyl cellulose, polyethylene terephthalate, and polymethylmethacrylate, to name but a few of the more common ones. Non-magnetizable metals, glass and numerous other materials having the general properties described above are also entirely suitable as base materials, provided that in each case a substance stable at the decomposition temperature is used.

20 As a general procedure, the base material is heated to decomposition temperature and exposed to the vapors of the carbonyl compound until a coating of the desired thickness has been deposited. The base material may be heated prior to the exposure and brought while still hot into contact with the vapors, but a preferable practice is to heat the base material at its surface while it is in contact with the vapors. For this purpose the base material may be heated by any one of numerous well-known methods, such as by being passed in contact with a heated surface, by high frequency electromagnetic energy or by 25 infrared radiation. Induction heating in the case of electrically conductive materials may also be employed.

25 A preferred procedure as applied to the formation of an iron coating on a base tape is described below with reference to the accompanying drawing showing schematically suitable apparatus in which the invention may be practiced.

30 The apparatus consists in general of an elongated chamber 10 having opposed slits 12 and 13 through which a tape to be coated may be run, and inlet and outlet conduits 14 and 15 by which an atmosphere of vapors of a carbonyl compound may be maintained within the chamber. A heating platen 16 having a smooth upper surface over which the tape is passed is mounted within the chamber with power leads 17 for the heating element 35 18 leading to a variable power source 20 by which the

temperature of the platen may be controlled. To prevent exposure of heated areas other than the top surface of the platen 16, insulation, as indicated at 21, may be provided around the top surface.

The operation of the apparatus consists in feeding the tape 22 through the chamber 10 and over the heating platen 16 while an atmosphere of carbonyl vapors is supplied to the chamber and while the temperature of the upper surface of the tape 22 is maintained above the decomposition temperature of the carbonyl compound.

In a typical operation for instance, an iron coating on a tape of regenerated cellulose may be formed by supplying the chamber 10 with iron pentacarbonyl vapors under atmospheric pressure at a temperature above 103° C. (the boiling point of iron pentacarboxyl), preferably at about 120° C., while heating the tape to between 160 and 200° C. A thin uniform homogeneous deposit of iron is thus formed by the reaction:



By introducing oxygen into the chamber in addition to the iron pentacarbonyl the iron may be deposited as 25 ferromagnetic iron oxide, according to the reaction



Although this invention has been described with reference to preferred embodiments, it is contemplated that 30 obvious modifications of its practice will occur to those skilled in the art, and that such may be made without departing from the scope of the invention.

Having thus disclosed this invention and described in detail preferred embodiments of it, I claim and desire to secure by Letters Patent:

5 1. The method of applying a ferromagnetic surface coating to a non-magnetizable base surface comprising heating said non-magnetizable base surface, and contacting said surface with an atmosphere comprising vapors of iron pentacarbonyl and oxygen, the temperature of the base surface while in contact with said atmosphere being above the decomposition temperature of the carbonyl compound, and the time of contact being such as to deposit a thin layer of ferromagnetic iron oxide suitable for magnetic recording on said base surface.

10 15 2. The method of applying a ferromagnetic surface coating to a non-magnetizable base surface comprising heating said non-magnetizable base surface and contacting said surface with an atmosphere comprising vapors of an iron carbonyl compound and oxygen, the temperature of the base surface while in contact with said atmosphere being above the decomposition temperature of the carbonyl compound, and the time of contact being such as to deposit a thin layer of ferromagnetic iron oxide suitable for magnetic recording on said base surface.

References Cited in the file of this patent

UNITED STATES PATENTS

|           |                  |       |               |
|-----------|------------------|-------|---------------|
| 2,041,480 | Oexmann          | ----- | May 19, 1936  |
| 2,616,165 | Brennan          | ----- | Nov. 4, 1952  |
| 2,619,433 | Davis et al.     | ----- | Nov. 25, 1952 |
| 2,671,034 | Steinfeld        | ----- | Mar. 2, 1954  |
| 2,698,812 | Schladitz        | ----- | Jan. 4, 1955  |
| 2,784,115 | Brinsmaid et al. | ----- | Mar. 5, 1957  |